

1,419,530.

W. WILSON.  
THERMIONICALLY ACTIVE SUBSTANCE.  
APPLICATION FILED AUG. 12, 1918.

Patented June 13, 1922.



Inventor:  
William Wilson  
by A. C. Barnes, Atty

# UNITED STATES PATENT OFFICE.

WILLIAM WILSON, OF EAST ORANGE, NEW JERSEY, ASSIGNOR TO WESTERN ELECTRIC COMPANY, INCORPORATED, OF NEW YORK, N. Y., A CORPORATION OF NEW YORK.

## TERMIONICALLY-ACTIVE SUBSTANCE.

1,419,530.

Specification of Letters Patent. Patented June 13, 1922.

Application filed August 12, 1918. Serial No. 249,523.

To all whom it may concern:

Be it known that I, WILLIAM WILSON, a subject of the King of Great Britain, residing at East Orange, in the county of 5 Essex, State of New Jersey, have invented certain new and useful Improvements in Thermionically-Active Substances, of which the following is a full, clear, concise, and exact description.

10 This invention relates to thermionically active substances which may serve as a source of electrons in a thermionic device, such as an audion. It has been known for some time that platinum filaments coated 15 with alkaline earth oxide have a high order of thermionic activity. An object of the present invention is to subject ductile metals of the iron group such as iron, nickel or cobalt to a special treatment whereby their 20 thermionic activity is increased and made comparable to that of oxide-coated platinum filaments.

As disclosed in the patent to Nicolson & Hull, No. 1,209,324, December 19, 1916— 25 electron emitting cathodes and the process of manufacturing the same, a platinum-coated filament having a high order of activity may be made by applying alternate coatings of carbonate or oxide of barium or 30 strontium, the coated filament being finally baked in the open air for about two hours. It has been discovered that if this process is applied to a metal of the iron group, while its activity may be increased, it is not 35 increased nearly as much as in the case where the coating is finally baked either (a) in absence of oxygen or (b) baked in air on the filament for a comparatively short period; for instance, from one to five 40 minutes.

It is desirable that clean or pure metal should be employed as the core or body of the filament and accordingly the metal of the iron group which is chosen, if not already 45 clean, may be cleaned by pre-glowing in vacuo, or in the absence of oxygen at a high temperature, and then coated. In the pre-glowing, a pressure which varies from .1 to .0001 mm. has been used. It is only 50 necessary to maintain the filament at a high or flashing temperature for a short time, viz, about five seconds.

After the filament has been pre-glowed, it is not essential that it be coated in the 55 particular way outlined above. For in-

stance, the filament may be coated by sputtering the coating material on the filament. This is done by placing the filament near the coating material, both being in vacuo. The coating material is heated and it sputters 60 and deposits on the hot filament.

When the filament is cleansed as indicated above by flashing in vacuo or in the absence of oxygen, occluded gases are driven out of the filament and any oxides that are on the filament are reduced. Best results are obtained if the filament is kept in this condition, and to this end, after the filament has been cleansed in this manner, all subsequent heating of the filament should be in vacuo or 65 in the absence of oxygen, to prevent re-oxidation and re-absorption of gasses. In certain cases it may be sufficient to perform the above process of flashing and baking in the absence of oxygen. It is not necessary 70 that the filament be cleaned as indicated above, and metal which has been rendered chemically pure by any other process may be used instead.

Apparatus that may be used in carrying 80 out both the pre-glowing and the sputtering processes, is shown in the figure of the drawing in which a boat 1 of molybdenum, for instance, contains the coating oxide or material 2 with which it is desired to coat the 85 filament 3. This coating material may be a mixture of strontium and barium oxides for instance. The boat 1 and the filament 3 are sealed into a glass tube 4, and may be heated electrically by current from the 90 sources of current 5 and 6, respectively. The glass tube 4 is provided with an outlet 7 through which it may be evacuated.

During evacuation of the glass tube, the filament and the boat are heated to a high 95 temperature, this pre-glowing serving to clean its surface thoroughly. The filament is then allowed to cool and the molybdenum boat heated to a high temperature (more than two thousand degrees C.). Some of 100 the coating material 2 sputters or evaporates and is condensed on the filament.

Another method which may be employed for coating the filament is as follows:

The metal which is to be employed as the 105 core or body of the filament should be obtained as metallurgically pure as possible. This metal is reduced to the form of a twisted filament as shown in the Nicolson-Hull Patent No. 1,209,324, supra, and as 110

disclosed therein, this filament may be suspended between two electrodes, for supplying current which passes through the filament to heat it. The filament is given a total of sixteen coats of carbonates of barium and strontium, applied in the following order:

- 10      4 coats of  $\text{SrCO}_3$ .  
       4 coats of  $\text{BaCO}_3$ .  
       4 coats of  $\text{SrCO}_3$ .  
       4 coats of  $\text{BaCO}_3$ .

15      Between the application of each coating, the wire should be flashed at a red heat and after the final coating has been applied the filament is baked in the open air for a short time, for instance, about three minutes, the temperature of the filament being low enough that only a relatively small amount of oxidation of the body or core of the 20 filament takes place.

25      The coating material may be applied in an aqueous solution as disclosed in Nic-  
       olson-Hull Patent No. 1,209,824, or paraffine may be used as a carrier for the coating  
       material as described and claimed in Hocker  
       application Serial No. 252,689, filed Septem-  
       ber 5, 1918. In this case the strontium car-  
       bonate and barium carbonate are thoroughly  
       mixed and stirred into separate batches of  
       30 paraffine. The stirring may be continued  
       until the paraffine is sufficiently cool to con-  
       geal, after which it may be worked into  
       small rods which can be placed upon suitable  
       holders for application to the heated fila-  
       35 ment. The paraffine melts on coming in con-  
       tact with the hot filament and a portion of  
       the alkaline earth compound is deposited  
       on the filament. Flashing the filament as  
       40 indicated above, during the coating process  
       serves to burn off the paraffine and to reduce

the carbonate to the oxide which adheres to the filament. First a paraffine rod containing strontium carbonate is employed to apply four coats to the filament, then a paraffine rod containing barium carbonate to 45 give four coats more, etc., until a suitable coating of the desired thickness has been provided.

50      A filament made as indicated above may be employed as the cathode of a thermionic amplifier connected as shown in the patent to Arnold, No. 1,129,942, March 2, 1915.

55      This application is a continuation in part of my copending application No. 182,965, filed July 26, 1917, for method of making thermionically active substances.

60      The apparatus described but not claimed in this application for coating a filament is claimed in the copending application of E. R. Stoekle, Serial No. 527,178, filed January 5, 1922.

65      What is claimed is:

1. A filament comprising a core of a ductile metal of the iron group and a coating of strontium and barium oxides, said filament having a degree of thermionic activity comparable to that of a platinum filament similarly coated and operated under similar conditions.

70      2. A filament comprising a core of nickel and a coating of strontium and barium oxides, said filament having a degree of thermionic activity comparable to that of a platinum filament similarly coated and operated under similar conditions.

75      In witness whereof, I hereunto subscribe my name this 6th day of August A. D., 1918.

WILLIAM WILSON.

### DISCLAIMER

1,419,530.—William Wilson, East Orange, N. J. THERMIONICALLY ACTIVE SUB-  
       STANCE. Patent dated June 13, 1922. Disclaimer filed May 16, 1934, by  
       the assignee, American Telephone and Telegraph Company.

Hereby enters this disclaimer to claim 2 of said Letters Patent, to wit:

“2. A filament comprising a core of nickel and a coating of strontium and barium oxides, said filament having a degree of thermionic activity comparable to that of a platinum filament similarly coated and operated under similar conditions.”

[Official Gazette June 5, 1934.]